



US007195531B2

(12) **United States Patent**  
Ito et al.

(10) **Patent No.:** US 7,195,531 B2  
(45) **Date of Patent:** Mar. 27, 2007

(54) **IMAGE DISPLAY UNIT AND METHOD FOR MANUFACTURING AN IMAGE DISPLAY UNIT**

(75) Inventors: **Takeo Ito**, Kumagaya (JP); **Tsuyoshi Oyaizu**, Fukaya (JP); **Takashi Nishimura**, Fukaya (JP); **Satoshi Koide**, Fukaya (JP); **Hitoshi Tabata**, Fukaya (JP)

(73) Assignee: **Kabushiki Kaisha Toshiba**, Tokyo (JP)

(\*) Notice: Subject to any disclaimer, the term of this patent is extended or adjusted under 35 U.S.C. 154(b) by 0 days.

(21) Appl. No.: 11/436,518

(22) Filed: May 19, 2006

(65) **Prior Publication Data**

US 2006/0211326 A1 Sep. 21, 2006

**Related U.S. Application Data**

(62) Division of application No. 10/487,625, filed as application No. PCT/JP02/08490 on Aug. 3, 2002, now Pat. No. 7,075,220.

(30) **Foreign Application Priority Data**

Aug. 24, 2001 (JP) ..... 2001-255204

(51) **Int. Cl.**

**H01J 9/22** (2006.01)

**H01J 1/62** (2006.01)

**H01J 63/04** (2006.01)

(52) **U.S. Cl.** ..... **445/11; 445/13; 445/24; 313/495; 313/496**

(58) **Field of Classification Search** ..... **445/9-13, 445/23, 24, 29, 31, 38-41; 313/461-466, 313/473, 481, 558-562, 553, 495-496**

See application file for complete search history.

(56)

**References Cited**

**U.S. PATENT DOCUMENTS**

|                   |         |                           |
|-------------------|---------|---------------------------|
| 5,453,659 A       | 9/1995  | Wallace et al.            |
| 5,866,978 A *     | 2/1999  | Jones et al. .... 313/495 |
| 6,278,233 B1      | 8/2001  | Sanou et al. .... 313/495 |
| 6,383,047 B1 *    | 5/2002  | Minami et al. .... 445/24 |
| 6,433,487 B1      | 8/2002  | Yamazaki .... 315/169.3   |
| 2001/0041490 A1 * | 11/2001 | Nomura et al. .... 445/24 |

**FOREIGN PATENT DOCUMENTS**

|    |             |         |
|----|-------------|---------|
| CN | 1134035 A   | 10/1996 |
| CN | 1298196 A   | 6/2001  |
| EP | 717429      | 6/1996  |
| EP | 1100107     | 5/2001  |
| JP | 2001-195982 | 7/2001  |

\* cited by examiner

*Primary Examiner*—Mariceli Santiago

*Assistant Examiner*—Christopher M. Raabe

(74) *Attorney, Agent, or Firm*—Oblon, Spivak, McClelland, Maier & Neustadt, P.C.

(57) **ABSTRACT**

An image display unit having a structure in which a heat-resistant fine particle layer is formed on a metal back layer disposed on a phosphor layer, and a getter layer is deposited/formed on the heat-resistant fine particle layer by vapor-depositing. The fine particle layer is desirably formed in a specified pattern, and a filmy getter layer is formed in a pattern complementary to the former pattern. The average particle size of heat-resistant fine particles which may use SiO<sub>2</sub>, TiO<sub>2</sub>, Al<sub>2</sub>O<sub>3</sub>, Fe<sub>2</sub>O<sub>3</sub> is 5 nm to 30  $\mu$ m. Since abnormal discharging is restricted, the destruction and deterioration of an electron emitting element and a phosphor screen are prevented to provide a high-brightness, high-grade display.

**8 Claims, 2 Drawing Sheets**



**FIG.1****FIG.2**

FIG.3



FIG.4



## 1

**IMAGE DISPLAY UNIT AND METHOD FOR  
MANUFACTURING AN IMAGE DISPLAY  
UNIT**

This is a Divisional application of and is based upon and claims the benefit of priority under 35 U.S.C. §120 from U.S. Ser. No. 10/487,625, filed Feb. 24, 2004; the entire content is incorporated herein by reference.

**TECHNICAL FIELD**

The present invention relates to an image display unit and a method for manufacturing an image display unit. More specifically, the invention relates to an image display unit having an electron source and a phosphor screen forming an image by irradiation of an electron beam emitted from the electron source within a vacuum envelope and a manufacturing method thereof.

**BACKGROUND ART**

An image display unit, which displays an image by irradiating an electron beam which is emitted from an electron source to a phosphor material to cause the phosphor material to emit light, generally has the electron source and the phosphor material within a vacuum envelope. When gas (surface adsorption gas) adsorbed to the inner surface of the vacuum envelope is separated to lower a degree of vacuum in the envelope, electrons emitted from the electron source are disturbed from reaching the phosphor material, and a high-brightness image display cannot be made. Therefore, it is necessary to keep the inside of the vacuum envelope under high vacuum.

The gas generated in the envelope is ionized by the electron beam and accelerated by an electric field to collide with the electron source, possibly damaging the electron source.

The conventional color cathode-ray tube (CRT) or the like retains a desired degree of vacuum by activating a getter material disposed in the vacuum envelope after sealing and adsorbing the gas released from the inner wall to the getter material during operation. And, it is now being attempted to apply the achievement of a high degree of vacuum and the retention of a degree of vacuum by the getter material to a flat type image display unit.

The flat type image display unit is provided with an electron source which has multiple electron emitting elements arranged on a flat substrate. The capacity of the vacuum envelope is considerably reduced as compared with that of an ordinary CRT, but the surface area of the wall releasing the gas does not be reduced. Therefore, when the surface adsorption gas in a volume similar to that of the CRT is released, deterioration of the degree of vacuum in the vacuum envelope becomes quite substantial. Accordingly, the getter material plays a very important role for the flat type image display unit.

Recently, formation of a layer of the getter material in an image display area is being studied. For example, Japanese Patent Laid-Open Application No. Hei 9-82245 discloses a flat type image display unit having a structure in which a thin film of a getter material having conductivity, such as titanium (Ti), zirconium (Zr) or the like, is overlaid on a metal layer (metal back layer) which is formed on a phosphor layer or the metal back layer itself is comprised of the getter material having the conductivity.

The metal back layer is aimed to enhance brightness by reflecting to the face plate side the light advancing toward the electron source in light emitted from the phosphor

## 2

material by the electrons emitted from the electron source, to play a role as an anode electrode by imparting conductivity to the phosphor layer, and to prevent the phosphor layer from being damaged by ions generated by ionization of the gas remained in the vacuum envelope.

The conventional field emission display (FED) had a disadvantage that an electric discharge (vacuum arc discharge) was easily caused when images were formed for a long period because a face plate having a phosphor screen

- 10 and a rear plate having an electron emitting element had a very small gap (space) of one to several millimeters between them, and a high voltage of about 10 kV was applied to the small gap to form a high electric field. And, when such an abnormal electric discharge occurred, a large discharge current in a range of several amperes to several hundred amperes flowed instantaneously, so that there was a possibility that the electron emitting element of a cathode section and the phosphor screen of an anode section were destructed or damaged.
- 20 Lately, it is proposed to form a gap section in the metal back layer being used as the anode electrode in order to ease the damage resulting from the occurrence of an abnormal electric discharge. An image display unit configured to have the metal back layer coated with a getter layer having conductivity is proposed to have a gap in the getter layer by forming the getter layer in a specified pattern in order to additionally restrict the occurrence of electric discharge so as to improve a withstand pressure characteristic.

Conventionally, as a method of forming the getter layer 30 having a specified pattern, there is proposed a method of disposing a mask having a pore pattern on a metal back layer and forming the getter layer by a vacuum-deposition method or a sputtering method. But, this method has disadvantages that patterning accuracy, pattern fineness and the like are limited, and an advantageous effect of preventing an electric discharge to improve the withstand pressure characteristic is not sufficient.

The present invention has been made to remedy the above 40 disadvantages and provides an image display unit capable of providing a high-brightness, high-grade display with electron emitting elements and a phosphor screen prevented from being destructed or deteriorated by electric discharge, and a manufacturing method thereof.

**SUMMARY OF THE INVENTION**

A first aspect of the present invention is an image display unit comprising a face plate, an electron source disposed to oppose the face plate, and a phosphor screen formed on the inner surface of the face plate, wherein the phosphor screen has a phosphor layer which emits light by an electron beam emitted from the electron source, a metal back layer formed on the phosphor layer, a heat-resisting fine particle layer formed on the metal back layer and a getter layer formed on the heat-resisting fine particle layer.

The image display unit can have the heat-resisting fine particle layer in a specified pattern and can have a filmy getter layer in an area, where the heat-resisting fine particle layer is not formed, on the metal back layer. And, the phosphor screen can have a light absorption layer for separating the individual phosphor layers, and the heat-resisting fine particle layer formed in at least a part of the area located above the light absorption layer.

And, the heat-resisting fine particles can have an average 60 particle size of 5 nm to 30  $\mu\text{m}$ . The heat-resisting fine particles can be fine particles of at least one type of metal oxide selected from a group consisting of  $\text{SiO}_2$ ,  $\text{TiO}_2$ ,  $\text{Al}_2\text{O}_3$

and  $\text{Fe}_2\text{O}_3$ . The getter layer can be a layer of at one type of metal selected from a group consisting of Ti, Zr, Hf, V, Nb, Ta, W and Ba or an alloy mainly consisting of such metals. Besides, the electron source can have plural electron emitting elements disposed on a substrate. Furthermore, the metal back layer can have a removed portion or a high resistance portion in prescribed regions.

A second aspect of the present invention is a method for manufacturing an image display unit comprising forming a phosphor screen, which has a phosphor layer and a metal back layer coated on the phosphor layer, on the inner surface of a face plate, and disposing the phosphor screen and an electron source in a vacuum envelope, further comprising forming a heat-resisting fine particle layer on the metal back layer, and a step of forming a layer of a getter material by vacuum-depositing the getter material on the metal back layer from above the heat-resisting fine particle layer.

The method for manufacturing an image display unit according to the second aspect can have forming a heat-resisting fine particle layer in a specified pattern on the metal back layer in the heat-resisting fine particle layer forming step, and forming a filmy getter layer in an area, where the heat-resisting fine particle layer is not formed, on the metal back layer. And, the phosphor screen can have a light absorption layer for separating the individual phosphor layers and the heat-resisting fine particle layer formed in at least a part of the area located above the light absorption layer on the metal back layer.

And, the heat-resisting fine particles can have an average particle size of 5 nm to 30  $\mu\text{m}$ . The heat-resisting fine particles can be fine particles of at least one type of metal oxide selected from a group consisting of  $\text{SiO}_2$ ,  $\text{TiO}_2$ ,  $\text{Al}_2\text{O}_3$  and  $\text{Fe}_2\text{O}_3$ . And, the getter material can be at least one type of metal selected from a group consisting of Ti, Zr, Hf, V, Nb, Ta, w and Ba or an alloy mainly consisting of such metals. Besides, the electron source can have plural electron emitting elements disposed on a substrate. Besides, forming the phosphor screen can comprise forming a metal back layer having a removed portion or a high resistance portion in prescribed regions.

The image display unit of the invention has a layer of the heat-resisting fine particles having a prescribed particle size (e.g., an average particle size of 5 nm to 30  $\mu\text{m}$ ) on the metal back layer of the phosphor screen and a layer of the getter material formed on the heat-resisting fine particle layer by, for example, vapor-depositing. The surface of the heat-resisting fine particle layer has fine unevenness because of the outside shapes of the fine particles, so that a film forming property of the getter material to be deposited on the layer becomes considerably poor. Therefore, a continuous uniform getter material film (getter film) is not formed on the heat-resisting fine particle layer, and the getter material is simply adhered/deposited. Therefore, the getter film is formed on only areas, where the heat-resisting fine particle layer is not formed, of the metal back layer.

And, because the getter film having the pattern is formed as described above, the occurrence of electric discharge is restricted and the peak value of a discharge current is suppressed if electric discharge occurs in especially a flat type image display unit such as the FED, so that the electron emitting elements or the phosphor screen is prevented from being destructed, damaged or deteriorated.

In the method for manufacturing an image display unit of the present invention, when a method of vapor-depositing the getter material from the above of the pattern of the heat-resisting fine particle layer after the heat-resisting fine particle layer is formed in a specified pattern is adopted, the

getter material-deposited film is formed on areas, where the heat-resisting fine particle layer is not formed, of the metal back layer, and the getter film having the pattern of the heat-resisting fine particle layer and the inversion pattern can be formed. And, by forming the getter film having the pattern as described above, especially the flat type image display unit such as the FED can restrict the occurrence of electric discharge and suppress the peak value of discharge current if electric discharge occurs, and the electron emitting elements or the phosphor screen can be prevented from being destructed, damaged or deteriorated.

And, the pattern of the heat-resisting fine particle layer can be formed in high fineness and high precision by a screen printing method or the like, so that the getter film in its reverse pattern can also be formed in high fineness and high precision.

#### BRIEF DESCRIPTION OF THE DRAWINGS

FIG. 1 is a sectional diagram showing a structure of a getter film-attached phosphor screen formed according to the first embodiment of the invention.

FIG. 2 is a sectional diagram showing part A of FIG. 1 in an enlarged form.

FIG. 3 is a sectional diagram schematically showing a structure of an FED having as an anode electrode the getter film-attached phosphor screen according to the first embodiment.

FIG. 4 is a sectional diagram showing a structure of the getter film-attached phosphor screen according to the second embodiment.

#### BEST MODE FOR CARRYING OUT THE INVENTION

Preferred embodiments of the invention will be described. It is to be understood that the invention is not limited to the following embodiments.

In the first embodiment, a light absorption layer made of a black pigment is first formed in a specified pattern (e.g., stripes) on the inner surface of a glass substrate which is to be a face plate by photolithography or a printing method. A  $\text{ZnS}$ -based,  $\text{Y}_2\text{O}_3$ -based or  $\text{Y}_2\text{O}_3\text{S}$ -based phosphor liquid is applied onto the light absorption layer by a slurry method or the like and dried, then patterning is made by the photolithography to form a three-color phosphor layer of red (R), green (G) and blue (B). The phosphor layer of individual colors can also be formed by a spray method or a printing method. When the spray method or the printing method is used, the patterning by the photolithography is also used, if necessary.

Then, a metal back layer is formed on the phosphor screen having the light absorption layer and the phosphor layer formed as described above. To form the metal back layer, there can be adopted, for example, a method by which a metal film of aluminum (Al) or the like is formed by vacuum-depositing on a thin film of an organic resin such as nitrocellulose formed by the spin method, and organic substances are removed by additional baking. The metal back layer can also be formed using a transfer film as described below.

The transfer film has a structure in that a metal film of Al or the like and an adhesive agent layer are superposed sequentially on a base film with the parting agent layer (and also a protective film, if necessary) intervening therebetween. This transfer film is disposed so to contact the adhesive agent layer with the phosphor layer and pressur-

ized. A stamp method, a roller method or the like is available as a pressing method. Thus, the transfer film is pressed to adhere the metal film, and the base film is peeled so as to transfer the metal film to the phosphor screen.

Then, a heat-resisting fine particle layer is formed on the metal back layer (metal film) formed as described above to have a specified pattern by a screen printing method or the like. The area where the heat-resisting fine particle layer pattern is formed can be determined on, for example, an area located on the light absorption layer. When the heat-resisting fine particle layer is formed in the above-described pattern avoiding the phosphor layer, there is an advantage that lowering of brightness because of the absorption of an electron beam from the electron source by the fine particle layer is small.

Material configuring the heat-resisting fine particles is not limited to a particular one but can be any type as long as it has insulating properties and can resist heating at a high temperature in a sealing step or the like. For example, fine particles of a metal oxide such as  $\text{SiO}_2$ ,  $\text{TiO}_2$ ,  $\text{Al}_2\text{O}_3$  or  $\text{Fe}_2\text{O}_3$  are available, and such metal oxides can be used alone or in a combination of two or more of them.

These heat-resisting fine particles desirably have an average particle size of 5 nm to 30  $\mu\text{m}$ , and more desirably 10 nm to 10  $\mu\text{m}$ . When the fine particles have an average particle size of less than 5 nm, the surface of the fine particle layer is substantially free from unevenness and very smooth. Thus, a getter material-deposited film is also formed uniformly without interruption on the heat-resisting fine particle layer. Therefore, a patterned getter film cannot be formed. When the fine particles have an average particle size of exceeding 30  $\mu\text{m}$ , it becomes impossible to form a heat-resisting fine particle layer.

Then, a metal back-attached phosphor screen where the heat-resisting fine particle layer is patterned is disposed together with the electron source in the vacuum envelope. There is adopted a method of forming a vacuum vessel by vacuum-sealing a face plate having the phosphor screen and a rear panel having the electron source such as plural electron emitting elements with flit glass or the like.

The getter material is then vapor-deposited from above the heat-resisting fine particle layer pattern in the vacuum envelope to form the getter material-deposited film in areas of the metal back layer where the heat-resisting fine particle layer is not formed. For the getter material, a metal selected from Ti, Zr, Hf, V, Nb, Ta, W and Ba, or an alloy mainly containing at least one of such metals.

Thus, a getter film 3 having a reverse pattern of a pattern of a heat-resisting fine particle layer 2 is formed on a metal back layer 1 of Al or the like as shown in FIG. 1. FIG. 1 shows a cross section of the metal back-attached phosphor screen formed according to the first embodiment. In FIG. 1, reference numeral 4 denotes a glass substrate, 5 denotes a light absorption layer, and 6 denotes a phosphor layer. FIG. 2 is an expanded view of part A of FIG. 1. In FIG. 2, reference numeral 7 denotes heat-resisting fine particles, and 8 denotes a getter material deposited on the heat-resisting fine particles 7.

After the getter material is deposited, the getter film 3 is kept retained in a vacuum atmosphere in order to prevent it from deteriorating. Therefore, it is desirable that, after the heat-resisting fine particle layer 2 is patterned on the metal back layer 1, the phosphor screen is disposed in the vacuum envelope, and the getter material is deposited in the vacuum envelope.

The structure of an FED having the phosphor screen on which the getter film is patterned is shown in FIG. 3. This

FED is configured in that a face plate 10 having a getter film-attached phosphor screen 9 and a rear plate 12 having multiple electron emitting elements 11, which are arranged in matrix, are disposed to oppose each other with a narrow gap (space) G of about one to several millimeters between them, and a high voltage of 5 to 15 kV is applied to the very small gap G between the face plate 10 and the rear plate 12.

Electric discharge (dielectric breakdown) occurs easily in the gap G between the face plate 10 and the rear plate 12 because the gap G is very small, but the peak value of discharge current is suppressed if an electric discharge occurs in the FED formed in the embodiment, and instantaneous concentration of energy is avoided. And, the electron emitting elements and the phosphor screen are prevented from being destructed, damaged or deteriorated because the maximum value of discharge energy is reduced.

It was described in the first embodiment that the structure had the metal back layer continuously formed without any gap or a separated part. But, the image display unit of the invention is not limited to the described structure. As the second embodiment, the metal back layer 1 may be cut or made to have high resistance at prescribed locations on the light absorption layer 5 or the like as shown in FIG. 4. Removed portions or high resistance portions 13 can be formed in the metal back layer 1 by a method of applying a liquid for dissolving or oxidizing the metal to the metal back layer 1, a method of cutting the metal back layer 1 by laser, or a method of forming a pattern of the metal back layer by depositing with a mask.

And, in the structure having conduction interrupted by the removed portions or the high resistance portions 13 of the metal back layer 1 as described above, electric discharge is further restricted and a withstand voltage characteristic is improved, so that an image having high brightness without suffering from deterioration of brightness can be obtained.

Then, specific examples of applying the invention to the FED will be described.

#### EXAMPLE 1

A light absorption layer (light-shielding layer) consisting of a black pigment was formed in a stripe form on a glass substrate by a photolithography, and a three color phosphor layer of red (R), green (G) and blue (B) was formed to have stripe patterns between the adjacent patterns of the light absorption layer by the photolithography. Thus, a phosphor screen having the light absorption layer and the phosphor layer with the specified patterns was formed.

Then, an Al film was formed as a metal back layer on the phosphor screen. Specifically, an organic resin solution mainly containing an acryl resin was applied to and dried on the phosphor screen to form an organic resin layer, an Al resin was formed thereon by vacuum-depositing, and heating was performed for baking at a temperature of 450°C. for 30 minutes so as to decompose and remove an organic component.

Next, a silica paste consisting of 5 wt % of silica ( $\text{SiO}_2$ ) fine particles (particle size of 10 nm), 4.75 wt % of ethyl cellulose and 90.25 wt % of butyl carbitol acetate was screen-printed on the Al film using a screen mask having openings at locations just above the light absorption layer. Thus, a pattern of the  $\text{SiO}_2$  layer was formed on an area just above the light absorption layer.

Ba was then deposited on the  $\text{SiO}_2$  layer in a vacuum atmosphere. As a result, Ba was deposited as the getter material on the  $\text{SiO}_2$  layer but did not form a uniform film. A uniform deposited film of Ba as the getter material was

formed on the areas, where the  $\text{SiO}_2$  layer was not formed, of the Al film. Thus, the getter film having a reverse pattern of the pattern of the  $\text{SiO}_2$  layer was formed on the Al film.

Surface resistivity of the getter film was measured in a state that a vacuum atmosphere was retained. The measured result is shown in Table 1.

An FED was produced by a common procedure using a panel having the patterned  $\text{SiO}_2$  layer, on which the getter film was not deposited, as a face plate. First, an electron generation source, which had multiple surface conduction type electron emitting elements formed in matrix on a substrate, was fixed to a glass substrate to produce a rear plate. Then, the rear plate and the above-described face plate were opposed to each other with a support frame and a spacer between them and sealed with flit glass to produce a vacuum envelope. The face plate and the rear plate had a gap of 2 mm between them. Subsequently, the vacuum envelope was evacuated, and Ba was deposited toward the panel surface (the metal back-attached phosphor screen with the patterned  $\text{SiO}_2$  layer formed) to form the getter film in the reverse pattern of the pattern of the  $\text{SiO}_2$  layer on the Al film.

The FED obtained by Example 1 was determined for evaluation of its withstand voltage characteristic by a common procedure. In addition, fineness of the getter film pattern and a degree of electrical disconnection between the patterns were examined. The determined results are shown in Table 1.

The withstand voltage characteristic of the FED was evaluated by:  $\odot$  indicating that a withstand voltage is high and a withstand voltage characteristic is quite good,  $\circ$  indicating that a withstand voltage characteristic is good,  $\Delta$  indicating that a withstand voltage characteristic is not good practically, and  $\times$  indicating that a withstand voltage characteristic is defective and impractical. Fineness of the getter film pattern was evaluated by:  $\odot$  indicating that the pattern has very high fineness,  $\circ$  indicating that fineness is high,  $\Delta$  indicating that fineness is low and is not good practically, and  $\times$  indicating that fineness is very low. A degree of electrical disconnection between patterns was evaluated by:  $\odot$  indicating that electrical disconnection between patterns is complete,  $\circ$  indicating that electrical disconnection is good,  $\Delta$  indicating that electrical disconnection is made somehow or other, and  $\times$  indicating that electrical disconnection is defective.

#### EXAMPLE 2

An Al film was formed on a phosphor screen formed in the same way as in Example 1, and a paste consisting of 10 wt % of  $\text{Al}_2\text{O}_3$  fine particles having a particle size of 7  $\mu\text{m}$ , 4.75 wt % of ethyl cellulose and 85.25 wt % of butyl carbitol acetate was screen-printed on the Al film to form a pattern of the  $\text{Al}_2\text{O}_3$  layer.

Then, Ba was deposited on the formed pattern of the  $\text{Al}_2\text{O}_3$  layer in the same way as in Example 1 to form a getter film (Ba film) having a reverse pattern of the pattern of the  $\text{Al}_2\text{O}_3$  layer. Surface resistivity of the getter film was measured in a state that a vacuum atmosphere was retained. The measured result is shown in Table 1.

Using a panel having the patterned  $\text{Al}_2\text{O}_3$  layer, on which the getter film was not deposited, as the face plate, an FED was produced in the same way as in Example 1. The withstand voltage characteristic of the obtained FED was determined for evaluation by a common procedure. And, fineness of the getter film pattern and a degree of electrical

disconnection between the patterns were examined in the same way as in Example 1. The determined results are shown in Table 1.

Besides, as Comparative Example 1, the getter film was formed on the entire surface of the Al film by depositing Ba on the Al film of the phosphor screen without forming a pattern of an  $\text{SiO}_2$  layer or an  $\text{Al}_2\text{O}_3$  layer as the heat-resisting fine particle layer. As Comparative Example 2, a pattern of the getter film was formed by depositing Ba on the Al film of the phosphor screen with a mask having openings in portions just above the phosphor layer interposed.

Then, surface resistivity of the getter films obtained in Comparative Examples 1 and 2 were measured in a state that a vacuum atmosphere was retained. And, using the panels, on which the getter films were not deposited, as the face plates, FEDs were produced in the same way as in Example 1. Withstand voltage characteristic of the obtained FEDs, fineness of the getter film patterns and a degree of electrical disconnection between the patterns were examined in the same way as in Example 1. The results are shown in Table 1.

TABLE 1

|                                               | Example 1                 | Example 2                                     | Comparative Example 1 | Comparative Example 2 |
|-----------------------------------------------|---------------------------|-----------------------------------------------|-----------------------|-----------------------|
| Heat-resisting fine particles (particle size) | $\text{SiO}_2$<br>(10 nm) | $\text{Al}_2\text{O}_3$<br>(7 $\mu\text{m}$ ) | None                  | None                  |
| Surface resistivity of getter film            | $10^4\Omega/\square$      | $10^4\Omega/\square$                          | $10^2\Omega/\square$  | $10^9\Omega/\square$  |
| Fineness of getter film pattern               | $\odot$                   | $\circ$                                       | $\times$              | —                     |
| Disconnection between getter film patterns    | $\circ$                   | $\circ$                                       | $\circ$               | —                     |
| Withstand voltage characteristic              | $\odot$                   | $\circ$                                       | $\Delta$              | $\times$              |

It is evident from the results shown in Table 1 that in Examples 1 and 2 the getter films having a pattern with remarkable fineness and favorable electrical disconnection were formed. And, the obtained getter films have higher surface resistance as compared with those of Comparative Examples, and FEDs having a good withstand voltage characteristic can be realized.

In the Examples described above, the direct vapor deposition method called a lacquer method was used to form the metal back layer, but the same effects can be obtained by using the transfer method to form the metal back layer.

#### INDUSTRIAL APPLICABILITY

As described above, the electrically divided getter layer can be formed readily on the metal back layer of the phosphor screen according to the present invention. And, the getter film having a very fine and highly accurate pattern can be formed, so that the peak value of discharge current can be suppressed in case of occurrence of electric discharge in a flat type image display unit such as the FED, and the electron emitting elements or the phosphor screen can be prevented from being destructed, damaged or deteriorated.

What is claimed is:

1. A method for manufacturing an image display unit comprising:  
forming a phosphor screen, which has a phosphor layer and a metal back layer coated on the phosphor layer, on the inner surface of a face plate, and

disposing the phosphor screen and an electron source in a vacuum envelope, further comprising:  
 forming a heat-resisting fine particle layer on the metal back layer, and  
 forming a layer of a getter material by vacuum-depositing the getter material on the metal back layer from above the heat-resisting fine particle layer.  
 2. The method for manufacturing an image display unit according to claim 1, wherein the heat-resisting fine particle layer is formed in a specified pattern on the metal back layer in the forming of the heat-resisting fine particle layer, and a 10  
 15  
 20  
 25  
 30  
 35  
 40  
 45  
 50  
 55  
 60  
 65  
 70  
 75  
 80  
 85  
 90  
 95  
 100  
 105  
 110  
 115  
 120  
 125  
 130  
 135  
 140  
 145  
 150  
 155  
 160  
 165  
 170  
 175  
 180  
 185  
 190  
 195  
 200  
 205  
 210  
 215  
 220  
 225  
 230  
 235  
 240  
 245  
 250  
 255  
 260  
 265  
 270  
 275  
 280  
 285  
 290  
 295  
 300  
 305  
 310  
 315  
 320  
 325  
 330  
 335  
 340  
 345  
 350  
 355  
 360  
 365  
 370  
 375  
 380  
 385  
 390  
 395  
 400  
 405  
 410  
 415  
 420  
 425  
 430  
 435  
 440  
 445  
 450  
 455  
 460  
 465  
 470  
 475  
 480  
 485  
 490  
 495  
 500  
 505  
 510  
 515  
 520  
 525  
 530  
 535  
 540  
 545  
 550  
 555  
 560  
 565  
 570  
 575  
 580  
 585  
 590  
 595  
 600  
 605  
 610  
 615  
 620  
 625  
 630  
 635  
 640  
 645  
 650  
 655  
 660  
 665  
 670  
 675  
 680  
 685  
 690  
 695  
 700  
 705  
 710  
 715  
 720  
 725  
 730  
 735  
 740  
 745  
 750  
 755  
 760  
 765  
 770  
 775  
 780  
 785  
 790  
 795  
 800  
 805  
 810  
 815  
 820  
 825  
 830  
 835  
 840  
 845  
 850  
 855  
 860  
 865  
 870  
 875  
 880  
 885  
 890  
 895  
 900  
 905  
 910  
 915  
 920  
 925  
 930  
 935  
 940  
 945  
 950  
 955  
 960  
 965  
 970  
 975  
 980  
 985  
 990  
 995  
 1000  
 1005  
 1010  
 1015  
 1020  
 1025  
 1030  
 1035  
 1040  
 1045  
 1050  
 1055  
 1060  
 1065  
 1070  
 1075  
 1080  
 1085  
 1090  
 1095  
 1100  
 1105  
 1110  
 1115  
 1120  
 1125  
 1130  
 1135  
 1140  
 1145  
 1150  
 1155  
 1160  
 1165  
 1170  
 1175  
 1180  
 1185  
 1190  
 1195  
 1200  
 1205  
 1210  
 1215  
 1220  
 1225  
 1230  
 1235  
 1240  
 1245  
 1250  
 1255  
 1260  
 1265  
 1270  
 1275  
 1280  
 1285  
 1290  
 1295  
 1300  
 1305  
 1310  
 1315  
 1320  
 1325  
 1330  
 1335  
 1340  
 1345  
 1350  
 1355  
 1360  
 1365  
 1370  
 1375  
 1380  
 1385  
 1390  
 1395  
 1400  
 1405  
 1410  
 1415  
 1420  
 1425  
 1430  
 1435  
 1440  
 1445  
 1450  
 1455  
 1460  
 1465  
 1470  
 1475  
 1480  
 1485  
 1490  
 1495  
 1500  
 1505  
 1510  
 1515  
 1520  
 1525  
 1530  
 1535  
 1540  
 1545  
 1550  
 1555  
 1560  
 1565  
 1570  
 1575  
 1580  
 1585  
 1590  
 1595  
 1600  
 1605  
 1610  
 1615  
 1620  
 1625  
 1630  
 1635  
 1640  
 1645  
 1650  
 1655  
 1660  
 1665  
 1670  
 1675  
 1680  
 1685  
 1690  
 1695  
 1700  
 1705  
 1710  
 1715  
 1720  
 1725  
 1730  
 1735  
 1740  
 1745  
 1750  
 1755  
 1760  
 1765  
 1770  
 1775  
 1780  
 1785  
 1790  
 1795  
 1800  
 1805  
 1810  
 1815  
 1820  
 1825  
 1830  
 1835  
 1840  
 1845  
 1850  
 1855  
 1860  
 1865  
 1870  
 1875  
 1880  
 1885  
 1890  
 1895  
 1900  
 1905  
 1910  
 1915  
 1920  
 1925  
 1930  
 1935  
 1940  
 1945  
 1950  
 1955  
 1960  
 1965  
 1970  
 1975  
 1980  
 1985  
 1990  
 1995  
 2000  
 2005  
 2010  
 2015  
 2020  
 2025  
 2030  
 2035  
 2040  
 2045  
 2050  
 2055  
 2060  
 2065  
 2070  
 2075  
 2080  
 2085  
 2090  
 2095  
 2100  
 2105  
 2110  
 2115  
 2120  
 2125  
 2130  
 2135  
 2140  
 2145  
 2150  
 2155  
 2160  
 2165  
 2170  
 2175  
 2180  
 2185  
 2190  
 2195  
 2200  
 2205  
 2210  
 2215  
 2220  
 2225  
 2230  
 2235  
 2240  
 2245  
 2250  
 2255  
 2260  
 2265  
 2270  
 2275  
 2280  
 2285  
 2290  
 2295  
 2300  
 2305  
 2310  
 2315  
 2320  
 2325  
 2330  
 2335  
 2340  
 2345  
 2350  
 2355  
 2360  
 2365  
 2370  
 2375  
 2380  
 2385  
 2390  
 2395  
 2400  
 2405  
 2410  
 2415  
 2420  
 2425  
 2430  
 2435  
 2440  
 2445  
 2450  
 2455  
 2460  
 2465  
 2470  
 2475  
 2480  
 2485  
 2490  
 2495  
 2500  
 2505  
 2510  
 2515  
 2520  
 2525  
 2530  
 2535  
 2540  
 2545  
 2550  
 2555  
 2560  
 2565  
 2570  
 2575  
 2580  
 2585  
 2590  
 2595  
 2600  
 2605  
 2610  
 2615  
 2620  
 2625  
 2630  
 2635  
 2640  
 2645  
 2650  
 2655  
 2660  
 2665  
 2670  
 2675  
 2680  
 2685  
 2690  
 2695  
 2700  
 2705  
 2710  
 2715  
 2720  
 2725  
 2730  
 2735  
 2740  
 2745  
 2750  
 2755  
 2760  
 2765  
 2770  
 2775  
 2780  
 2785  
 2790  
 2795  
 2800  
 2805  
 2810  
 2815  
 2820  
 2825  
 2830  
 2835  
 2840  
 2845  
 2850  
 2855  
 2860  
 2865  
 2870  
 2875  
 2880  
 2885  
 2890  
 2895  
 2900  
 2905  
 2910  
 2915  
 2920  
 2925  
 2930  
 2935  
 2940  
 2945  
 2950  
 2955  
 2960  
 2965  
 2970  
 2975  
 2980  
 2985  
 2990  
 2995  
 3000  
 3005  
 3010  
 3015  
 3020  
 3025  
 3030  
 3035  
 3040  
 3045  
 3050  
 3055  
 3060  
 3065  
 3070  
 3075  
 3080  
 3085  
 3090  
 3095  
 3100  
 3105  
 3110  
 3115  
 3120  
 3125  
 3130  
 3135  
 3140  
 3145  
 3150  
 3155  
 3160  
 3165  
 3170  
 3175  
 3180  
 3185  
 3190  
 3195  
 3200  
 3205  
 3210  
 3215  
 3220  
 3225  
 3230  
 3235  
 3240  
 3245  
 3250  
 3255  
 3260  
 3265  
 3270  
 3275  
 3280  
 3285  
 3290  
 3295  
 3300  
 3305  
 3310  
 3315  
 3320  
 3325  
 3330  
 3335  
 3340  
 3345  
 3350  
 3355  
 3360  
 3365  
 3370  
 3375  
 3380  
 3385  
 3390  
 3395  
 3400  
 3405  
 3410  
 3415  
 3420  
 3425  
 3430  
 3435  
 3440  
 3445  
 3450  
 3455  
 3460  
 3465  
 3470  
 3475  
 3480  
 3485  
 3490  
 3495  
 3500  
 3505  
 3510  
 3515  
 3520  
 3525  
 3530  
 3535  
 3540  
 3545  
 3550  
 3555  
 3560  
 3565  
 3570  
 3575  
 3580  
 3585  
 3590  
 3595  
 3600  
 3605  
 3610  
 3615  
 3620  
 3625  
 3630  
 3635  
 3640  
 3645  
 3650  
 3655  
 3660  
 3665  
 3670  
 3675  
 3680  
 3685  
 3690  
 3695  
 3700  
 3705  
 3710  
 3715  
 3720  
 3725  
 3730  
 3735  
 3740  
 3745  
 3750  
 3755  
 3760  
 3765  
 3770  
 3775  
 3780  
 3785  
 3790  
 3795  
 3800  
 3805  
 3810  
 3815  
 3820  
 3825  
 3830  
 3835  
 3840  
 3845  
 3850  
 3855  
 3860  
 3865  
 3870  
 3875  
 3880  
 3885  
 3890  
 3895  
 3900  
 3905  
 3910  
 3915  
 3920  
 3925  
 3930  
 3935  
 3940  
 3945  
 3950  
 3955  
 3960  
 3965  
 3970  
 3975  
 3980  
 3985  
 3990  
 3995  
 4000  
 4005  
 4010  
 4015  
 4020  
 4025  
 4030  
 4035  
 4040  
 4045  
 4050  
 4055  
 4060  
 4065  
 4070  
 4075  
 4080  
 4085  
 4090  
 4095  
 4100  
 4105  
 4110  
 4115  
 4120  
 4125  
 4130  
 4135  
 4140  
 4145  
 4150  
 4155  
 4160  
 4165  
 4170  
 4175  
 4180  
 4185  
 4190  
 4195  
 4200  
 4205  
 4210  
 4215  
 4220  
 4225  
 4230  
 4235  
 4240  
 4245  
 4250  
 4255  
 4260  
 4265  
 4270  
 4275  
 4280  
 4285  
 4290  
 4295  
 4300  
 4305  
 4310  
 4315  
 4320  
 4325  
 4330  
 4335  
 4340  
 4345  
 4350  
 4355  
 4360  
 4365  
 4370  
 4375  
 4380  
 4385  
 4390  
 4395  
 4400  
 4405  
 4410  
 4415  
 4420  
 4425  
 4430  
 4435  
 4440  
 4445  
 4450  
 4455  
 4460  
 4465  
 4470  
 4475  
 4480  
 4485  
 4490  
 4495  
 4500  
 4505  
 4510  
 4515  
 4520  
 4525  
 4530  
 4535  
 4540  
 4545  
 4550  
 4555  
 4560  
 4565  
 4570  
 4575  
 4580  
 4585  
 4590  
 4595  
 4600  
 4605  
 4610  
 4615  
 4620  
 4625  
 4630  
 4635  
 4640  
 4645  
 4650  
 4655  
 4660  
 4665  
 4670  
 4675  
 4680  
 4685  
 4690  
 4695  
 4700  
 4705  
 4710  
 4715  
 4720  
 4725  
 4730  
 4735  
 4740  
 4745  
 4750  
 4755  
 4760  
 4765  
 4770  
 4775  
 4780  
 4785  
 4790  
 4795  
 4800  
 4805  
 4810  
 4815  
 4820  
 4825  
 4830  
 4835  
 4840  
 4845  
 4850  
 4855  
 4860  
 4865  
 4870  
 4875  
 4880  
 4885  
 4890  
 4895  
 4900  
 4905  
 4910  
 4915  
 4920  
 4925  
 4930  
 4935  
 4940  
 4945  
 4950  
 4955  
 4960  
 4965  
 4970  
 4975  
 4980  
 4985  
 4990  
 4995  
 5000  
 5005  
 5010  
 5015  
 5020  
 5025  
 5030  
 5035  
 5040  
 5045  
 5050  
 5055  
 5060  
 5065  
 5070  
 5075  
 5080  
 5085  
 5090  
 5095  
 5100  
 5105  
 5110  
 5115  
 5120  
 5125  
 5130  
 5135  
 5140  
 5145  
 5150  
 5155  
 5160  
 5165  
 5170  
 5175  
 5180  
 5185  
 5190  
 5195  
 5200  
 5205  
 5210  
 5215  
 5220  
 5225  
 5230  
 5235  
 5240  
 5245  
 5250  
 5255  
 5260  
 5265  
 5270  
 5275  
 5280  
 5285  
 5290  
 5295  
 5300  
 5305  
 5310  
 5315  
 5320  
 5325  
 5330  
 5335  
 5340  
 5345  
 5350  
 5355  
 5360  
 5365  
 5370  
 5375  
 5380  
 5385  
 5390  
 5395  
 5400  
 5405  
 5410  
 5415  
 5420  
 5425  
 5430  
 5435  
 5440  
 5445  
 5450  
 5455  
 5460  
 5465  
 5470  
 5475  
 5480  
 5485  
 5490  
 5495  
 5500  
 5505  
 5510  
 5515  
 5520  
 5525  
 5530  
 5535  
 5540  
 5545  
 5550  
 5555  
 5560  
 5565  
 5570  
 5575  
 5580  
 5585  
 5590  
 5595  
 5600  
 5605  
 5610  
 5615  
 5620  
 5625  
 5630  
 5635  
 5640  
 5645  
 5650  
 5655  
 5660  
 5665  
 5670  
 5675  
 5680  
 5685  
 5690  
 5695  
 5700  
 5705  
 5710  
 5715  
 5720  
 5725  
 5730  
 5735  
 5740  
 5745  
 5750  
 5755  
 5760  
 5765  
 5770  
 5775  
 5780  
 5785  
 5790  
 5795  
 5800  
 5805  
 5810  
 5815  
 5820  
 5825  
 5830  
 5835  
 5840  
 5845  
 5850  
 5855  
 5860  
 5865  
 5870  
 5875  
 5880  
 5885  
 5890  
 5895  
 5900  
 5905  
 5910  
 5915  
 5920  
 5925  
 5930  
 5935  
 5940  
 5945  
 5950  
 5955  
 5960  
 5965  
 5970  
 5975  
 5980  
 5985  
 5990  
 5995  
 6000  
 6005  
 6010  
 6015  
 6020  
 6025  
 6030  
 6035  
 6040  
 6045  
 6050  
 6055  
 6060  
 6065  
 6070  
 6075  
 6080  
 6085  
 6090  
 6095  
 6100  
 6105  
 6110  
 6115  
 6120  
 6125  
 6130  
 6135  
 6140  
 6145  
 6150  
 6155  
 6160  
 6165  
 6170  
 6175  
 6180  
 6185  
 6190  
 6195  
 6200  
 6205  
 6210  
 6215  
 6220  
 6225  
 6230  
 6235  
 6240  
 6245  
 6250  
 6255  
 6260  
 6265  
 6270  
 6275  
 6280  
 6285  
 6290  
 6295  
 6300  
 6305  
 6310  
 6315  
 6320  
 6325  
 6330  
 6335  
 6340  
 6345  
 6350  
 6355  
 6360  
 6365  
 6370  
 6375  
 6380  
 6385  
 6390  
 6395  
 6400  
 6405  
 6410  
 6415  
 6420  
 6425  
 6430  
 6435  
 6440  
 6445  
 6450  
 6455  
 6460  
 6465  
 6470  
 6475  
 6480  
 6485  
 6490  
 6495  
 6500  
 6505  
 6510  
 6515  
 6520  
 6525  
 6530  
 6535  
 6540  
 6545  
 6550  
 6555  
 6560  
 6565  
 6570  
 6575  
 6580  
 6585  
 6590  
 6595  
 6600  
 6605  
 6610  
 6615  
 6620  
 6625  
 6630  
 6635  
 6640  
 6645  
 6650  
 6655  
 6660  
 6665  
 6670  
 6675  
 6680  
 6685  
 6690  
 6695  
 6700  
 6705  
 6710  
 6715  
 6720  
 6725  
 6730  
 6735  
 6740  
 6745  
 6750  
 6755  
 6760  
 6765  
 6770  
 6775  
 6780  
 6785  
 6790  
 6795  
 6800  
 6805  
 6810  
 6815  
 6820  
 6825  
 6830  
 6835  
 6840  
 6845  
 6850  
 6855  
 6860  
 6865  
 6870  
 6875  
 6880  
 6885  
 6890  
 6895  
 6900  
 6905  
 6910  
 6915  
 6920  
 6925  
 6930  
 6935  
 6940  
 6945  
 6950  
 6955  
 6960  
 6965  
 6970  
 6975  
 6980  
 6985  
 6990  
 6995  
 7000  
 7005  
 7010  
 7015  
 7020  
 7025  
 7030  
 7035  
 7040  
 7045  
 7050  
 7055  
 7060  
 7065  
 7070  
 7075  
 7080  
 7085  
 7090  
 7095  
 7100  
 7105  
 7110  
 7115  
 7120  
 7